

Feb. 17, 1948.

J. C. CRAWFORD

2,435,957

TRIPACK FILMS WITH EMULSION LAYERS ADJACENT EACH  
OTHER AND METHOD OF MAKING SAME

Filed June 22, 1944



FIG 1



FIG 2



FIG 3

Inventor

JACK C CRAWFORD

By

W. Glenn Jones

Attorney

## UNITED STATES PATENT OFFICE

2,435,957

TRIPACK FILM WITH EMULSION LAYERS  
ADJACENT EACH OTHER AND METHOD  
OF MAKING SAMEJack C. Crawford, United States Navy,  
Anacostia, D. C.

Application June 22, 1944, Serial No. 541,557

3 Claims. (Cl. 95—2)

(Granted under the act of March 3, 1883, as  
amended April 30, 1928; 370 O. G. 757)

1

This invention relates to a photographic film, and more particularly to a film incorporating a plurality of light sensitive emulsion layers, adapted to the production of pictures in natural colors.

The term "film," as employed herein, refers to the article as a whole, embodying one or more transparent base reinforcing layers, and the light sensitive emulsion layers emplaced thereon.

Films are available on the market today which contain either one or two distinct emulsion layers. However, no truly satisfactory film of the so-called "tri-pack" type has as yet been proposed. Such a film incorporates three distinct light sensitive emulsion layers, one being blue sensitive, the next green sensitive and the other red sensitive, or panchromatic. The difficulties which to date have prevented the development of a successful tri-pack are largely mechanical in nature. The problem is to support all three of the emulsion layers on the film base without the employment of intervening layers of other material, the arrangement of the emulsion layers being such that the image formed in each upon exposure may thereafter be fixed upon an individual supporting base without loss of registry or impairment of the image. Experience has shown that the placing of even the thinnest of supporting layers between the emulsion layers distorts the light rays entering the next adjacent emulsion layer, with resulting loss in sharpness of definition.

It is an object of this invention to overcome the aforesaid and other difficulties and to supply a satisfactory tri-pack film. A further object is to supply a film of this type wherein the emulsion layers are placed adjacent each other without intervening supporting layers. Still another object is to provide a tri-pack film so arranged that the image formed in each of the three light sensitive emulsion layers upon exposure of the film, may be fixed or joined to an individual supporting base in such fashion as later to permit the picture to be printed in natural colors without loss of registry and with sharpness of image.

It is my invention that the foregoing objects may be attained by an arrangement whereby three light sensitive emulsion layers are sandwiched together between two transparent bases of Celluloid or like material, as illustrated in Fig. 1 of the accompanying drawings, wherein:

Fig. 1 is a cross sectional view, to an enlarged scale, taken through one edge of the film;

Fig. 2 is a cross sectional view, to an enlarged scale, taken through one edge of the blue sensitive layer and its transparent base support, the emulsion having been separated from the adja-

2

cent green sensitive emulsion layer during an initial step of processing the film for development; and

Fig. 3 is a cross sectional view, to an enlarged scale, taken through one edge of the green and red sensitive emulsion layers and showing each emulsion layer being joined to a transparent base support, the green sensitive emulsion layer having been joined to its base support after the removal of the emulsion from the developing and stop solutions.

In the drawings, the transparent support bases 10 and 11 are positioned at the front and rear sides of the film respectively (Fig. 1). By the front side of the film is meant the side through which the light first enters, as shown by the arrow in Fig. 1. The transparent supporting layers are usually composed of Celluloid or of a suitable transparent plastic material.

In fabricating the film, the blue sensitive emulsion layer 12, containing a yellow dye, is coated on the inner surface of the base 10. The yellow dye serves to prevent the light rays in the blue portion of the spectrum from penetrating the blue sensitive emulsion layer to more than a slight depth, with the result that the modification of the silver particles in this emulsion layer caused by exposing the film is confined to the region of the emulsion adjacent the film base 10. This condition is favorable to the formation of a good silver gelatin relief image from this portion of the film. The support 10, with the applied emulsion layer 12, forms the front element of the film.

A red sensitive, or panchromatic, emulsion layer 13, which is last exposed to the light, is coated in similar fashion on the inner, or frontward, surface of the base member 11. This emulsion layer 13 is then desensitized downwardly in suitable manner, as by the application of a potassium iodide solution to the frontward surface 13a. This method is disclosed by Seymour in U. S. Patent No. 1,946,640. As a result of this treatment, the silver particles in emulsion layer 13 which are modified on exposure are those which are located at or near the boundary between the emulsion and the base member 11, thus making it possible to form a good relief image with reference to this emulsion layer.

A green sensitive emulsion layer 14, containing a red dye, is then coated on top of the red sensitive emulsion layer 13 after the latter has been subjected to the desensitization treatment. The red dye acts as a filter for the following red sensitive, or panchromatic, emulsion layer 13, and it

also restrains the green light from penetrating deeply into the emulsion layer 14. Accordingly, the exposure in the emulsion layer 14 is held to the surface regions thereof adjacent the emulsion layer 12, this condition being that desired for forming a good silver gelatin relief image from the green sensitive emulsion layer. It may be noted that this second, or green sensitive, emulsion layer is coated in manufacture directly on the following panchromatic, or red sensitive, layer, and that it thereby forms an integral part of the rear element of the film.

The outer surface of the base support 11, or the back of the film, is preferably provided with a removable anti-halation coating 15 which serves to improve the quality of the image. This coating may be removed in the usual fashion during the developing process.

The front and rear elements of the film are then connected to each other by joining the open sides of the blue sensitive and the green sensitive emulsion layers by means of a suitable adhesive 16. The thickness of this adhesive layer is so small as to be hardly perceptible, and it causes no distortion of the light rays passing through it. The strength of the bond formed by the adhesive should be less than that existing either between the emulsion layer 12 and the base member 10, or between the emulsion layers 13 and 14 or the emulsion 13 and its support 11. Further, the strength of the adhesive should be such that while the emulsion layers 12 and 14 are held firmly together by it under normal conditions of usage of the film, the front and rear elements of the film may readily be peeled apart by hand during the processing of the exposed film. It has been found that polyvinyl acetate provides an adhesive bond of satisfactory character for this purpose, though other substances now known and used in similar fashion in the art would perform equally well.

In certain instances it may be possible to eliminate the use of the adhesive where the front and rear film elements may otherwise be held together in a satisfactory manner during exposure of the film. For example, the film components may be held firmly together between glass plates applied to the outer surfaces of the base supports 10 and 11.

When the film is used, it is exposed in the normal fashion. After exposure, the blue sensitive emulsion layer is peeled away from the green sensitive emulsion layer at the adhesive boundary. Each of the two resulting film strips is then developed. In the latter step, I prefer to employ a tanning developer incorporating sodium sulphate, as this type of solution prevents swelling of the gelatin and keeps it in good condition for transfer. A developing solution which I have found to be satisfactory has the following composition, solution B being added to solution A on making up and using the developer:

## A

|                          |       |     |    |
|--------------------------|-------|-----|----|
| Water                    | cc    | 500 | 65 |
| Citric acid              | grams | 1   |    |
| Pyro                     | do    | 6   |    |
| Hydroquinone             | do    | 4   |    |
| Methyl p-aminophenol     | do    | 1   |    |
| Sodium sulfate (20% sol) | cc    | 500 | 70 |

## B

|                             |       |       |    |
|-----------------------------|-------|-------|----|
| Sodium carbonate            | grams | 150   |    |
| Potassium bromide (10% sol) | cc    | 10    |    |
| Water                       | cc    | 1,000 | 75 |

After development the films are placed for about two minutes in a short stop bath such as a solution of 5% by weight boric acid in water, after which the two portions of the film may be exposed to light without harm. The above steps are carried out in a dark room under suitable conditions of light.

As the next step in the process, a third base support 17, see Fig. 3, carrying on one side a suitable sub to receive the silver image from the green sensitive emulsion layer, is soaked in water and is squeegeed down onto the surface of the green sensitive emulsion layer, the side of the base support 17 carrying the sub being placed adjacent the emulsion. In a few minutes the resulting film portion incorporating the green and red sensitive emulsion layers is submerged in hot water for a period, usually about 1 to 5 minutes, in order to dissolve the unhardened gelatin lying between the base layers 11 and 17. The latter are then pulled apart, leaving the green relief image on the new support 17 and the red relief image adhering to its original base 11.

All three of the base supports 10, 11 and 17 are then washed free of any remaining unhardened gelatin with hot water, after which the images thereon are fixed in an acid hardening fixing bath, and then washed and dried.

The resulting film strips are termed negative relief images. The processes for making three color transparencies or three color prints on paper from the negative relief images are well known in the art and need not here be described. The details of such procedures are fully described in various publications, one such publication, for example, being that of the Eastman Kodak Company, Rochester, New York, entitled "Color Printing, with Eastman Wash-Off Relief Film."

The invention described herein may be manufactured and used by or for the Government of the United States of America for governmental purposes without the payment of any royalties thereon or therefor.

Other modifications and changes in the number and arrangement of the parts may be made by those skilled in the art without departing from the nature of the invention, within the scope of what is hereinafter claimed.

I claim:

1. As a new article of manufacture, a tri-pack film consisting of two elements; the first element comprising a transparent reinforcing base through which the light first enters the film, and a blue sensitive emulsion layer, containing a yellow dye, coated on the inner surface thereof; and the second element comprising a rear transparent supporting member forming the back of the film, said rear supporting member having an anti-halation material applied to its rearward surface, and having a panchromatic emulsion layer coated on its frontward surface, said panchromatic layer being desensitized downwardly from its frontward surface by suitable treatment, and a green sensitive emulsion layer, containing a red dye, coated on said desensitized panchromatic emulsion layer; the two elements being joined together by a polyvinyl acetate adhesive of such characteristics that the elements of the film can be readily peeled apart by hand during development of the film, the juncture being effected between the open sides of the blue sensitive and the green sensitive emulsion layers.

2. In a method of making a film incorporate three light sensitive emulsion layers, the steps comprising applying a first emulsion layer to the

rearward surface of a front transparent supporting member; applying a second emulsion layer to the frontward surface of a rear transparent supporting member; desensitizing downwardly from its frontward surface said second emulsion layer; coating a third emulsion layer upon the frontward surface of said desensitized emulsion layer; applying a polyvinyl acetate adhesive to the rearward surface of said first emulsion layer and the frontward surface of said third emulsion layer, and joining said adhesive coated surfaces to form a unitary structure, the joint so formed being susceptible of rupture during the development process.

3. In a method of making a film incorporating three light sensitive emulsion layers, the steps comprising applying to the rearward surface of a front transparent supporting member as a first emulsion layer, a blue sensitive emulsion containing a yellow dye; applying to the frontward surface of a rear transparent supporting member as a second emulsion layer, a panchromatic emulsion; desensitizing downwardly from its frontward surface said second emulsion layer; coating upon the frontward surface of said desensitized emulsion layer as a third emulsion layer, a green

sensitive emulsion containing a red dye; and bonding together with polyvinyl acetate the film components so formed, said bond being formed between the rearward surface of said first emulsion layer and the frontward surface of said third emulsion layer.

JACK C. CRAWFORD.

#### REFERENCES CITED

10 The following references are of record in the file of this patent:

#### UNITED STATES PATENTS

|    | Number    | Name              | Date          |
|----|-----------|-------------------|---------------|
| 15 | 927,244   | Ives              | July 6, 1909  |
|    | 1,248,139 | Lawshe            | Nov. 27, 1917 |
|    | 1,261,542 | Ives              | Apr. 2, 1918  |
|    | 1,306,904 | Ives              | June 17, 1919 |
|    | 1,889,030 | Ball              | Nov. 29, 1932 |
| 20 | 1,946,640 | Seymour           | Feb. 13, 1934 |
|    | 1,951,043 | Weaver            | Mar. 13, 1934 |
|    | 1,966,653 | Thornton          | July 17, 1934 |
|    | 2,112,226 | Baldsiefen et al. | Mar. 29, 1938 |
|    | 2,177,342 | Hesser et al.     | Oct. 24, 1939 |
|    | 2,183,394 | Gaspar            | Dec. 12, 1939 |
|    | 2,316,294 | Sease             | Apr. 13, 1943 |